

# UNITED STATES PATENT OFFICE.

HEINRICH WACHWITZ, OF NUEREMBERG, GERMANY.

## METAL-WELDING.

SPECIFICATION forming part of Letters Patent No. 684,479, dated October 15, 1901.

Application filed May 9, 1898. Serial No. 680,141. (No specimens.)

To all whom it may concern:

Be it known that I, HEINRICH WACHWITZ, a subject of the Emperor of Germany, residing at Nuremberg, Bavaria, Germany, have invented certain new and useful Improvements in Processes for Plating Aluminium Sheets with Copper and other Metals, of which the following is a specification.

It has been found that plating aluminium with metals, and especially copper, by the usual process of heating or welding, an aluminium alloy is formed on the surface, which destroys the ductility of the copper coating-sheet (where copper is used) and prevents a perfect union between the aluminium plate and the coating metal where other metals than copper are used. The object of my invention is to overcome this twofold difficulty, and I accomplish it in the following manner.

In plating aluminium with copper I first form on the surface of the copper an alloy with zinc by coating the copper with said metal in liquid form and heating the coated plates and excluding the air during such heating. When the zinc-copper alloy has been so formed on the copper plates, the latter are hammered into thin sheets of aluminium in any suitable manner which will secure the firm application of the thin sheets of aluminium to or incorporated with the previously zinc-treated surface of the copper plates. The compound plate thus formed—*i.e.*, the zinc-treated copper plates incorporated with the thin aluminium covering—is then used to plate or coat the aluminium base, plate, or object, the aluminium-covered surface of the copper plate being placed contiguous to the aluminium base. This last step is performed by heating, rolling, and working in the manner described in United States Letters Patent No. 655,212, or by any method preferred.

When metals other than copper are used

to plate the aluminium, it is not necessary to use the zinc or form an alloy on the coating-body; but the hammered application of the thin sheet of aluminium to the coating-body preliminary to the regular plating by heat is essential and in all other respects, except as to the alloy, the process is the same.

It will be seen that my process ordinarily involves two steps—one mechanical (the hammering of the thin sheet of aluminium) and the other chemical and mechanical (the heating, rolling, and working); but when a plating of copper on aluminium is desired it involves three steps—chemical, (forming an alloy on the surface of the copper plate,) mechanical, (hammering the thin sheets of aluminium on the copper plates,) and chemical and mechanical, (heating, rolling, and working.)

Having thus described my invention, I claim and desire to obtain by Letters Patent—

1. The process of coating aluminium sheets with other metals, consisting of applying to the surface of the coating metal by hammering, a thin sheet or layer of aluminium, then applying said compound sheet to the aluminium sheet or body to be coated, and heating, rolling and working the same together.

2. The process of coating aluminium sheets or bodies with sheets of copper consisting in forming a zinc-copper alloy on the surface of the copper sheet, hammering the latter into a thin sheet of aluminium, then applying said compound sheet to the aluminium body to be coated, and heating, rolling, and working the same together.

In testimony whereof I affix my signature in presence of two witnesses.

HEINRICH WACHWITZ.

Witnesses:

ALEX WIELE,  
MAX SCHNEIDER.